

# UNITED STATES PATENT OFFICE.

JAMES R. ROSE, OF EDGEWORTH, PENNSYLVANIA, AND JOHN HARRIS, OF LAKEWOOD, OHIO, ASSIGNORS TO CARBO-OXYGEN COMPANY, OF PITTSBURGH, PENNSYLVANIA, A CORPORATION OF DELAWARE.

## GASEOUS FUEL.

1,404,232.

Specification of Letters Patent. Patented Jan. 24, 1922.

No Drawing.

Application filed December 26, 1919. Serial No. 347,459.

To all whom it may concern:

Be it known that we, (1) JAMES R. ROSE and (2) JOHN HARRIS, citizens of the United States, residing at (1) Edgeworth, (2) Lakewood, in the county of (1) Allegheny, (2) Cuyahoga, and State of (1) Pennsylvania, (2) Ohio, have invented a certain new and useful Improvement in Gaseous Fuel, of which the following is a full, clear, and exact description.

This invention relates to gaseous fuel, and particularly to fuels for the cutting and welding of metal wherein a combustible base of hydrogen is employed together with another gas or gases capable of producing within the blow pipe flame, a luminous cone whereby the application of the flame to the work is facilitated.

It has been proposed to mix with hydrogen gases such as illuminating gas and carbon monoxide, the mixture being particularly well suited for certain kinds of work. It is the purpose of this invention to produce a gas employing hydrogen as a combustible base which shall be particularly useful for the cutting of alloys, cast steel, corroded, dirty and slaggy iron and steel, as well as cast iron; also for heating large masses or bodies of metal for the purpose of softening the same. For this purpose we employ a mixture of butane and propane with hydrogen in proportions of from  $2\frac{1}{2}\%$  to  $12\frac{1}{2}\%$  by volume each of such butane and propane to the hydrogen constituent. By the use of this mixture, a high carbon content in the mixture is obtained, thereby producing a flame, the volume and heat units of which will be increased over the volume and heat units produced by the combustion of hydrogen alone with oxygen, to the extent to which the butane and propane are present in the mixture. The presence of the butane and propane in the mixture enables the metal to be pre-heated quickly and, in the

case of large masses or bodies of such metal, with sufficient rapidity to more than offset the loss of heat through conduction and radiation. This renders the fuel particularly useful for the cutting and heating of such heavy masses of metal, as well as for cutting the special metals of the character set forth hereinbefore.

According to Richards on Metallurgical Calculations, published in 1908, the flame temperature produced by the combustion of the aforesaid gases will exceed  $3200^{\circ}$  C., and the variations in the percentage of the said gases will cause the following variations in the net B. T. U. per cubic foot of mixture and in the cubic feet of oxygen required for the combustion of a cubic foot of such mixture:

No. 1 mixture, 95% H. with  $2\frac{1}{2}\%$  each of butane and propane; net B. T. U.'s 421; cu. ft. of oxygen .713.

No. 2 mixture, 75% H. with  $12\frac{1}{2}\%$  each of butane and propane; net B. T. U.'s 932; cu. ft. of oxygen 1.863.

Having thus described our invention, what we claim is:—

1. A gas for cutting, welding and heating purposes consisting of a mixture of butane and propane with hydrogen in the proportions of from  $2\frac{1}{2}\%$  to  $12\frac{1}{2}\%$  by volume each of butane and propane to hydrogen.

2. A gas for cutting, welding and heating purposes consisting of a mixture of butane and propane with hydrogen in proportions not substantially less than 5% by volume of such combined gases to the hydrogen and not materially more than 25% of such combined gases to the hydrogen, the butane and propane being present in the proportions of at least  $2\frac{1}{2}\%$  each in such mixture.

In testimony whereof, we hereunto affix our signatures.

JAMES R. ROSE.  
JOHN HARRIS.